

Dec. 29, 1925.

1,567,967

H. MACAUX

PROCESS OF GASIFYING AND CARBONIZING COAL AND LIKE FUEL SUBSTANCES

Filed Oct. 3, 1922



Inventor  
Henri Macaux  
by *H. Williamson & Co.*  
Attorneys

## UNITED STATES PATENT OFFICE.

HENRI MACAUX, OF PARIS, FRANCE, ASSIGNOR TO SOCIETE LYONNAISE DES EAUX ET DE L'ECLAIRAGE, OF PARIS, FRANCE.

## PROCESS OF GASIFYING AND CARBONIZING COAL AND LIKE FUEL SUBSTANCES.

Application filed October 3, 1922. Serial No. 592,076.

To all whom it may concern:

Be it known that I, HENRI MACAUX, a citizen of the Republic of France, and residing at Paris, Seine Department, in the Republic of France, have invented certain new and useful Processes of Gasifying and Carbonizing Coal and like Fuel Substances, of which the following is a specification.

In the methods employed in coke producing plants and gas works, the usual practice is to decompose at a red heat into carbon and free hydrogen a considerable percentage of the hydrocarbons contained in the coal or set free during the heating treatment of the same, and this affords as a rule a gas containing fifty volumes of free hydrogen per one hundred volumes of lighting gas. This decomposition increases with the amount of coal under the heating treatment and with the time of said treatment which varies from four to fifty hours during which the heat is transmitted from the outside to the centre of the mass. The hydrocarbon gas which is produced within the mass is caused to pass through the envelope of coke at a red heat which is already formed, and the gas is decomposed into its elements upon contact with the same. The above is the object of coking processes in which the maximum yield in weight of coke is to be obtained.

But the contrary result may be sought for, and especially in city gas works. While obtaining a marketable or available coke, it is proposed to volatilize the maximum amount of carbon in combination with the hydrogen from coal or the additional hydrogen which may be produced by the decomposition of water vapour by coke or may be obtained from a suitable outside source.

The process according to the present invention is adapted to obtain these results. In the said process, coal in a finely divided state is projected in a continuous manner into a chamber heated to redness which receives a continuous supply of hydrogen in the pure state or mixed with other gases and chiefly with water gas obtained by the decomposition of water by coke at a red heat, the hydrogen supply being in all cases so regulated, that its partial tension in the atmosphere of the chamber shall be greater than what would result from the dissociation of the hydrocarbons contained in the projected particles of coal or would be formed by their decomposition by

heat. The partial tension of the hydrogen supplied from the outside thus produced and maintained in the said chamber will act to prevent the dissociation of the substances of the coal into hydrogen and carbon, and on the other hand, by a continuous injection of coal in a very finely divided state, one will obtain the gasifying of its volatile parts if not in an instantaneous manner, at least at a very rapid rate and in proper progression.

The major part of the gasifying is thus effected in a fraction of a second instead of during several hours or period of ten hours as in the known methods, and it is rapidly completed upon the surface of the walls and of the mass of coke in formation. The temperature of the hydrogenation gas will progressively increase so as to act at the beginning of the trajectory of the particles of coal to produce the hydrogenation of their non-saturated constituents and then their pyrolytic decomposition into hydrocarbon gas in an excess of hydrogen. The gas thus obtained is directly discharged without being filtered through a layer of coke heated to redness. But the fineness of the particles, and the speed, and force of projection of the stream of coal powder are regulated so that in the residual particles of the coal upon contact of the same with the red hot walls of the chamber or with the already formed coke, will retain the binding parts which are necessary for the agglomeration of the coke in formation, and the latter may be increased by the compression due to the impact.

The said process can thus be used for the removal of the adhesive parts of classes of coals which are too rich in volatile substances to produce coke of the metallurgic grade. As concerns the shape and the temperature of the chambers used for the heating process, the practice which is current in gas or coke plants can be followed. The size of the coal particles may be for example that of the extra fine Carmaux coal which will pass through a 100 mesh sieve and the particles can be projected by centrifugal force or by like means, or by the effect of gravity alone; the volume of the hydrogenation gas supplied may for example be equal to the volume of coal gas which would be obtained by the current methods in the same chambers or retorts, so that calculation may

be made, for a given chamber or retort, of the respective outputs of the coal stream and the injected hydrogenation gas. Pressures in the chambers are adjusted at the extraction outlets as in the known methods.

The hydrogenation gas can be produced in the chambers or retorts themselves, when these become filled with red hot coke at the end of the treatment, and the resulting gas 10 may be injected into other chambers or retorts wherein the treatment is taking place, or the said gas can also be produced at the outside by special generators. But it is advisable to obtain the maximum percentage of hydrogen in this gas. It can be heated before injection by any suitable means.

The accompanying drawing shows by way of example a vertical section of a form of 20 construction of furnace with horizontal chamber, but obviously the process is also applicable to chambers or retorts of the vertical or the inclined type.

1 indicates a furnace chamber whose 25 walls are heated to redness. The coal in very fine powder is placed in a hopper 2 and delivered into said chamber by a centrifugal projector 3 which is mounted at one end of the latter. 4-4 indicates the 30 path of the coal particles. The hydrogenation gas supplied by a conduit 5, and the produced gas is discharged at the other end by the conduit 6. The coke mass is shown at 7 at a certain time during its formation; 35 towards the end of the process, the forward slope of said mass is near the point 8. The

ends of said chamber are closed by the doors 9, and when open they enable the use of a pusher 10 in order to dispose the coke mass upon the quenching surface 11.

The top of said chamber may be provided with the usual feeding passages 12. Before reaching the conduit 5, the hydrogenation gas may be heated by circulating it through a chamber filled with red hot coke 45 which is reaching the end of the heating stage, or through a regeneration device of a known type containing piled bricks or employing transmission of heat through the walls.

#### Claim—

A process for the gasifying of coal and like fuel, which consists in the continuous insufflation of finely divided coal into 55 chambers heated to redness, in the simultaneous injection into these chambers during the whole time the process is carried out, of a supplementary gas containing hydrogen and in such a proportion that the partial tension of the hydrogen shall be constantly 60 maintained at a higher degree than the tension which would result from the disassociation of the hydrocarbons contained in the coal and disengaged by the pyrolytic decomposition of the coal, and in evacuating the 65 gases produced without allowing the same to traverse a layer of red hot coke, for the purposes set forth.

In testimony that I claim the foregoing as my invention, I have signed my name.

HENRI MACAUX.